

# United States Patent Office

2,879,230

Patented Mar. 24, 1959

1

2,879,230

## MOTOR LUBRICATING OIL COMPOSITION

Stanley R. Newman, Robert Y. Heisler, and Kenneth L. Dille, Fishkill, and Norman Alpert, Poughkeepsie, N.Y., assignors to The Texas Company, New York, N.Y., a corporation of Delaware

No Drawing. Application November 19, 1956  
Serial No. 622,772

6 Claims. (Cl. 252—51.5)

This invention relates to motor lubricants containing a novel class of additives which reduce or suppress deposit formation in combustion engines. More specifically, this invention discloses that superior lubricating oils, from the standpoint of removal of low temperature deposits, are obtained by the addition thereto of a minor amount of a polyglycol carbamate of a prescribed composition.

As automobile manufacturers annually raise the compression ratio of their engines in the race for higher horsepower, the problem of engine deposits resulting from the fuel becomes increasingly more severe. Engine deposits which find their origin in the fuel are primarily responsible for surface ignition phenomena such as preignition and octane requirement increase (ORI) which is the tendency of spark ignition engines in service to require higher octane fuels for proper performance. There are two avenues by which this problem can be attacked. One approach is through the fuel and the other is through the lubricating oil. In a coassigned copending application filed of even date, Serial No. 622,809, now Patent No. 2,842,433, it is disclosed that superior hydrocarbon fuels from the standpoint of engine deposits result from the incorporation of a polyglycol carbamate of a prescribed composition. The present invention involves the discovery that the addition of a polyglycol carbamate to a lubricating oil produces lubricants marked by the ability to maintain a clean engine even with dirty fuels under low temperature conditions of operation.

Modern lubricating oils for internal combustion engines usually contain a combination of additives which impart detergent and dispersant properties as well as resistance to oxidation to lubricating oils. The detergent and dispersant properties are normally obtained by the addition of alkaline earth metal petroleum sulfonates, alkaline earth metal salts of alkyl-substituted aromatic compounds or derivatives of these compounds. The most commonly used anti-oxidant and inhibitor is a divalent metal dialkyl dithiophosphate. Lubricating oils containing additives of these types are compounded to a supplement I level. Oils of supplement I level are very satisfactory lubricants for modern automobile engines from all standpoints with the exception of effectiveness in controlling deposits formed under low temperature conditions. The lubricating compositions of this invention are particularly designed for control of deposits resulting at low temperature conditions of operation.

The improved lubricating oils of this invention contain a polyglycol carbamate ester of the general formula:



wherein R is hydrogen, an alkyl, alkenyl, or alkynyl group having from 1 to 18 carbon atoms, R' is an alkyl, alkenyl, or alkynyl group having from 1 to 18 carbon atoms, and n ranges from 2 to 6, in an amount sufficient

2

to reduce deposit formation in the engine. The polyglycol carbamate ester is effective in the motor lubricant in concentrations as low as 0.25 volume percent but concentrations of 0.5 to 3.0 volume percent are normally employed. There is no critical upper limit of concentration, but economic considerations dictate that concentrations less than 5.0 volume percent of the polyglycol carbamate ester be present in the lubricating oil.

The present invention also includes the method of operating an internal combustion engine which comprises utilizing a fuel containing a polyglycol carbamate ester of the following general formula:



wherein R is hydrogen or an alkyl, alkenyl or alkynyl radical having from 1 to 18 carbon atoms, R' is an alkyl, alkenyl or alkynyl radical having from 1 to 18 carbon atoms and n ranges from 2 to 6, said compound being present in the fuel and engine lubricant in amounts sufficient to suppress the formation of engine deposits.

The range in which the polyglycol carbamate may be used in the fuel in the process of this invention is from 0.01 volume percent up to about 1 volume percent, preferably from about 0.04 to 0.3 volume percent. The addition range of polyglycol carbamate in the engine lubricant of the process of the invention is from 0.25 to 5.0 volume percent and preferably from 0.5 to 3 volume percent in the oil.

Polyglycol carbamates of the present invention include for example: diethylene glycol bis (N,N-diallyl carbamate); diethylene glycol bis [N,N-di-(1-methylisopentyl) carbamate]; diethylene glycol bis (N-2-ethylhexyl carbamate); diethylene glycol bis (N,N-dipropargyl carbamate); diethylene glycol bis (N-allyl carbamate); diethylene glycol bis (N-n-propyl carbamate); diethylene glycol bis (N,N-diisobutyl carbamate); triethylene glycol bis (N,N-diallyl carbamate); triethylene glycol bis (N,N-dioctadecyl carbamate); triethylene glycol bis [N-(1,1-dimethyl-2-propynyl) carbamate]; tetraethylene glycol bis (N-2-ethylhexyl carbamate); tetraethylene glycol bis (N-allyl carbamate); pentaethylene glycol bis (N-propargyl carbamate); pentaethylene glycol bis (N-n-propyl carbonate) hexaethylene glycol bis (N,N-diallyl carbamate); hexaethylene glycol bis (N-n-butyl carbamate); and hexaethylene glycol bis (N-2-ethylhexyl carbamate).

The polyglycol carbamate esters which inhibit the deposit-forming tendencies of hydrocarbon fuels are readily formed by a series of reactions involving the formation of a polyglycol dichloroformate and thereafter reacting said dichloroformate with an aliphatic hydrocarbon amine. The reaction product is then separated from the unreacted substances by known purification steps. The preparation of the polyglycol dichloroformate type compound is disclosed in U.S. Patents 2,370,567 and 2,370,569.

The following examples are given to demonstrate the preparation of the esters of the invention.

### EXAMPLE I

#### Preparation of diethylene glycol bis (N-allyl carbamate)

737 g. (12.94 moles) of allyl amine and 1115 g. (14.11 moles) of pyridine were placed in a five liter flask equipped with a stirrer, a condenser, a thermocouple probe, and an addition funnel, and the mixture was cooled to 50° F. 1360 g. (5.88 moles) of diethylene glycol dichloroformate was added to the mixture to yield a brick red solution lightening somewhat as a salt was

formed. One liter of benzene was added to the mixture, which was then stirred for about 48 hours after which one liter of water was added. The oil-water layers were separated and the oil layer was washed with 10 percent hydrochloric acid and then washed again with a saturated salt solution several times until the washes were neutral. The solution was then filtered, and the benzene and water were removed by distillation at atmospheric pressure. The residue, 1369 g., was crystallized to a waxy solid of low melting point. This solid was recrystallized from ether to yield 991 g. of white crystals having a melting point of 50 to 53° F. The theoretical analysis for diethylene glycol bis (N-allyl carbamate) shows the compound to have 53.0 percent carbon; 7.36 percent hydrogen, and 10.0 percent nitrogen. The actual analysis of the compound formed in accordance with this example showed it to have 52.7 percent carbon; 7.37 percent hydrogen; and 9.8 percent nitrogen. The yield of the purified componnd was 62 percent of the theoretical yield.

## EXAMPLE II

*Preparation of diethylene glycol bis(N-2-ethylhexyl carbamate)*

193 ml. (2.4 moles) of pyridine and 354 ml. (2.2 moles) of 2-ethylhexylamine were placed in a liter, triple-necked flask equipped with a stirrer, condenser, thermometer, and addition funnel. This mixture was stirred and maintained below 50° F. while 231 g. (1 mole) of diethylene glycol dichloroformate were slowly added. The solution changed from yellow to green to brown and finally to dark red. After about 15 hours of stirring, 500 ml. of ether was added and the resulting mixture was washed 5 times, each time with 400 ml. of 10 percent hydrochloric acid followed by 4 washes with 300 ml. of saturated salt solution per wash. The neutral water insoluble layer was dried over anhydrous calcium sulfate. The calcium sulfate was next removed by filtration and the ether removed by vacuum distillation. The crude product of 350 g. was dissolved in benzene and twice passed through synthetic magnesium silicate to give a light orange solution. The benzene was removed by vacuum distillation. The product had a calculated analysis of 63.4 percent carbon; 10.54 percent hydrogen; 6.74 percent nitrogen; and a molecular weight of 416. An actual analysis of the product showed 62.2 percent carbon; 10.4 percent hydrogen; 6.6 percent nitrogen; and a molecular weight of 402.

## EXAMPLE III

*Preparation of diethylene glycol bis(N-n-propyl carbamate)*

865 g. of n-propylamine and 1290 ml. of pyridine were placed into a 5 liter, triple-neck flask equipped with stirrer, condenser, thermometer and addition funnel. This mixture was stirred and maintained below 50° F. while 1556 g. (6.73 moles) of diethylene glycol dichloroformate were slowly added. 800 ml. of benzene were added to the mixture to keep the reaction mobile and then the mixture was stirred for about 5 hours. The crude product-benzene solution was then washed 3 times with 800 ml. of a 10 percent hydrochloric acid solution followed by 3 washes with 1000 ml. of water. The crude product was further purified by a synthetic magnesium silicate percolation, and the benzene was evaporated to give approximately 700 g. of the crude product. The product was again dissolved in benzene and decolorized by passing through decolorizing charcoal and cooled to recover 330 g. of white crystals. A small sample was dried over  $P_2O_5$  at 65° F. under 2 mm. pressure. The product had a theoretic 52.1 percent carbon, 8.7 percent hydrogen, 10.12 percent nitrogen, and a molecular weight of 276. The actual analysis of the compound showed it to have 51.8 percent carbon, 7.5 percent hydrogen, and 9.9 percent nitrogen.

## EXAMPLE IV

*Preparation of diethylene glycol bis (N,N-diallyl carbamate)*

970 g. of diallylamine, 500 ml. of benzene, and 880 ml. of pyridine were placed into a triple-neck flask equipped with a stirrer, condenser, thermometer, and addition funnel. The mixture was stirred and maintained below 50° F. while 1155 g. of diethylene glycol dichloroformate were slowly added. After stirring for about 15 hours, the mixture was washed with a 10 percent hydrochloric acid solution and thereafter washed again with a saturated salt solution. The remaining benzene and water were removed by distillation. The crude product weighed 1580 g. Further purification was made by vacuum distillation. Analysis of the fraction boiling at 173 to 195° F. at 300 to 750 microns was made. This product theoretically had 61.1 percent carbon; 7.95 percent hydrogen; and 7.95 percent nitrogen. Actual analysis of this compound show it contained 60.6 percent carbon; 7.95 percent hydrogen; and 7.8 percent nitrogen.

The lubricating oil of this invention is effective in maintaining deposits at a low level with the results that an engine lubricated therewith shows exceptionally clean cylinder head, combustion space, valves and ring belt area. The low deposit level in the engine minimizes surface ignition in all its manifestations, mainly preignition and "knock." In addition, the low deposit level reduces the engine's octane requirement increase. Deposits on surfaces contacted by the additive-containing lubricating oil, such as piston skirts and cylinder walls, are very markedly reduced.

The polyglycol carbamates of this invention are effective in controlling deposit formation in lubricants employed in spark ignition engines, diesel motors and gas turbines. However, they are normally used in motor oils for spark ignition engines wherein fuel derived deposits formed during low temperature operation are a particularly vexing problem. Diesel lubricants containing these polyglycol carbamates are effective in eliminating deposits resulting from the use of the so-called "economy" diesel fuels, e. g., fuels having a high sulfur content or containing cracked or residual stocks. The polyglycol carbamates are also useful as deposit-control additives in gas turbine lubricants which are generally ester base lubricants. They are also useful in aviation oils which lubricate reciprocating aviation engines. The scope of the lubricating oils to which the polyglycol carbamates of the invention are added with the formation of superior lubricants from the standpoint of deposit-removal is broad and includes mineral oils, synthetic lubricating oils and mixtures thereof.

The hydrocarbon mineral oils usable in the invention can be paraffin base, naphthene base or mixed paraffin-naphthene base distillate or residual oils. Paraffin base distillate lubricating oil fractions are used in the formulation of premium grade motor oils such as are contemplated in this invention. The lubricating base generally has been subjected to solvent refining to improve its lubricity and viscosity temperature relationship as well as solvent dewaxing to remove waxy components and improve the pour of the oil. Broadly speaking, mineral lubricating oils having an SUS viscosity at 100° F. between 50 and 1,000 may be used in the formulation of the improved lubricants of this invention but usually the viscosity range falls between 70 and 300 at 100° F.

The mineral lubricating oils to which the additives of this invention are added usually contain other additives designed to impart other desirable properties thereto. For example, V.I. improvers, such as the polymethacrylates, are normally included therein as are materials which act as detergents and dispersants for the removed combustion chamber deposits.

The V.I. improver normally used is a polymethacrylate of the general formula:



wherein R is an aliphatic radical ranging from butyl to stearyl and n is an integer.

The most commonly used detergent-dispersant additive is an alkaline earth metal petroleum sulfonate such as calcium petroleum sulfonate or barium petroleum sulfonate. These products are so well known as detergent-dispersant additives they require no further description. Similarly, divalent metal alkyl phenolates are widely used as detergents either alone or in combination with the alkaline earth metal petroleum sulfonates.

The most commonly used inhibitor and anti-oxidant is a divalent metal alkyl dithiophosphate which results from the neutralization of a  $\text{P}_2\text{S}_5$ -alcohol reaction product with a divalent metal or divalent metal oxide. The most widely used inhibitors are barium and zinc alkyl dithiophosphates.

The synthetic lubricating bases are usually of the ester or ether type. High molecular weight, high boiling liquid aliphatic dicarboxylic acid esters possess excellent viscosity-temperature relationships and lubricating properties and are finding ever increasing utilization in lube oils adapted for high and low temperature lubrication; esters of this type are used in the formulation of jet engine oils. Examples of this class of synthetic lubricating bases are the diesters of acids such as sebacic, adipic, azelaic, alkenylsuccinic, etc. Specific examples of these diesters are di-2-ethylhexyl sebacate, di-2-ethylhexyl azelate, di-2-ethylhexyl adipate, di-n-amyl sebacate, di-2-ethylhexyl n-dodecyl succinate, di-2-ethoxyethyl sebacate, di-2'-methoxy-2-ethoxyethyl sebacate (the methyl Carbitol diester), di-2'-ethyl-2-n-butoxyethyl sebacate (the 2-ethylbutyl Cellosolve diester), di-2-n-butoxyethyl azelate (the n-butyl Cellosolve diester) and di-2'-n-butoxy-2-ethoxyethyl-n-octyl succinate (the n-butyl Carbitol diester).

Polyester lubricants formed by a reaction of an aliphatic dicarboxylic acid of the type previously described, a glycol and a monofunctional aliphatic monohydroxy alcohol or an aliphatic monocarboxylic acid in specified mole ratios are also employed as the synthetic lubricating base in the compositions of this invention; polyesters of this type are described in U.S. 2,628,974. Polyesters formed by reaction of a mixture containing specified amounts of dipropylene glycol, sebacic acid and 2-ethylhexanol and of a mixture containing adipic acid, diethylene glycol and 2-ethylhexanoic acid illustrate this class of synthetic polyester lubricating bases.

Polyalkylene ethers as illustrated by polyglycols are also used as the lubricating base in the composition of this invention. Polyethylene glycol, polypropylene glycol, polybutylene glycols and mixed polyethylene-polypropylene glycols are examples of this class of synthetic lubricating bases.

The sulfur analogs of the above-described diesters, polyesters and polyalkylene esters are also used in the formulation of the lubricating compositions of this invention. Dithioesters are exemplified by di-2-ethylhexyl thiosebacate and di-n-octyl thiodipropionate; polyethylene thioglycol is an example of the sulfur analogs of the polyalkylene glycols; sulfur analogs of polyesters are exemplified by the reaction product of adipic acid, thioglycol and 2-ethylhexyl mercaptan.

The action of the polyglycol carbamates of this invention in improving the deposit-removing properties of a lubricating oil was demonstrated by a modified Chevrolet deposits test—CRC FL-2-650. The laboratory engines were operated under the standard conditions of this test with the exception that crankcase oil temperatures were 10° F. lower, the water jacket temperatures were 5° F. 75

lower, and the crankcases of the test engines were ventilated. These modifications were in every case in the direction of making the test more severe and were intended to simulate low temperature conditions wherein 5 deposit formation is most pronounced. After the termination of each run, the engine was disassembled and its parts evaluated by a merit system adapted from the CRC-L-4-1252 test. This merit system involved visual examination of the engine parts in question and their 10 rating according to deposits by comparison with standards which had assigned ratings. For example, a rating of 10 on piston skirt designated a perfectly clean piston while a rating of zero represented the worst condition. Similarly, a rating of 100 on total engine deposits represented 15 a perfectly clean engine, etc.

The fuel used in this test was a high quality regular grade gasoline comprising a mixture of thermal cracked stock, fluid catalytically cracked stock and straight run gasoline. This regular base fuel had an 87.0 ASTM 20 research octane rating, contained 2.90 ml. of TEL per gallon, had an API gravity of 58.0 and a boiling range between 106° F. and 396° F.; the base fuel was negative in the copper corrosion test and had an oxidation stability in the ASTM test of 530 minutes minimum. 25 The reference fuel also contained minor amounts of gasoline inhibitors, namely, N,N'-di-secondary butyl-p-phenylene diamine, lecithin, and N,N'-disalicylidene 1,2-diamino propane.

The reference lubricating oil was a 20-20W heavy 30 duty oil meeting supplement I requirements. This reference oil contained a methacrylate V.I. improver and a balanced combination of additives which impart detergent, dispersant and anti-oxidant properties to the oil. The additive mixture comprised a barium petroleum 35 sulfonate, and a zinc alkyl dithiophosphate in which the alkyl group is a methylcyclohexyl radical.

In the following table the results obtained in the modified Chevrolet deposits test with lubricating oils having the additives of the invention therein are shown. In 40 these experiments the concentration of additive in the lubricant was determined at the conclusion of the run by analysis.

TABLE I

|                                                       | Piston Skirt | Total Engine Deposits | Concentration Of Additive In Oil At Run Termination, Vol. Percent |
|-------------------------------------------------------|--------------|-----------------------|-------------------------------------------------------------------|
| Reference Oil                                         | 6.1          | 79.9                  | 0                                                                 |
| Reference Oil plus DEG, bis(N-2-ethylhexyl carbamate) | 8.0          | 88.0                  | 3                                                                 |
| Reference Oil plus DEG, bis(N,N-diallyl carbamate)    | 8.0          | 88.0                  | 5                                                                 |

DEG=diethylene glycol.

It is evident from the results shown in the above table that the compounds of the invention are very effective deposit suppressors.

60 The following table sets forth the results of the method of operating a combustion engine wherein the additive of the invention is carried to the combustion chamber in both the fuel and the engine lubricant. The base fuel and the base lubricant were those described as used in the above-described Chevrolet S-II test.

TABLE II.—CHEVROLET S-II TEST RESULTS

|                                                                                                                                | Piston Skirt Rating | Total Engine Rating |
|--------------------------------------------------------------------------------------------------------------------------------|---------------------|---------------------|
| Reference Fuel and Reference Oil                                                                                               | 6.1                 | 80.1                |
| Reference fuel and 0.05 vol. % DEG bis(N,N-diallyl carbamate) and Reference oil plus 1.0 vol. % DEG bis(N,N-diallyl carbamate) | 8.0                 | 88.0                |

The great improvement in engine cleanliness as demonstrated by the result obtained in the above deposits test proves the merit of the method of operating a combustion engine in accordance with the present invention.

Obviously, many modifications and variations of the invention, as hereinbefore set forth, may be made without departing from the spirit and scope thereof, and therefore only such limitations should be imposed as are indicated in the appended claims.

We claim:

1. A lubricating oil containing a minor amount of a polyglycol carbamate having the following general formula:



wherein R is selected from the group consisting of hydrogen, alkyl, alkenyl and alkynyl radicals having from 1 to 18 carbon atoms, R' is selected from the group consisting of alkyl, alkenyl and alkynyl radicals having from 1 to 18 carbon atoms, and n ranges from 2 to 6, in an amount sufficient to reduce engine deposits.

2. The lubricating composition of claim 1 wherein R is hydrogen.

3. The lubricating composition of claim 1 wherein n is 2.

4. A lubricating oil as described in claim 1 wherein the amount of polyglycol carbamate present in the base fluid is from 0.25 to 5.0 volume percent.

5. A mineral lubricating oil containing from 0.5 to 3.0 volume percent of diethylene glycol bis(N,N-diallyl carbamate).

6. A mineral lubricating oil containing from 0.5 to 3.0 volume percent of diethylene glycol bis(N-2-ethylhexyl carbamate).

15 **References Cited in the file of this patent**

**UNITED STATES PATENTS**

|           |            |               |
|-----------|------------|---------------|
| 2,161,615 | Dietrich   | June 6, 1939  |
| 2,438,452 | Pollock    | Mar. 23, 1948 |
| 2,528,399 | Strain     | Oct. 31, 1950 |
| 2,657,984 | Brathwaite | Nov. 3, 1953  |

**OTHER REFERENCES**

"Motor Oils and Engine Lubrication," Georgi, Reinhold Pub. Corp. (1950), pages 337-342.